

[54] SPUN-LIKE YARN AND METHOD OF MANUFACTURING SAME

[75] Inventors: Hiroshi Edagawa; Ituo Nakamura; Kozo Susami, all of Otsu, Japan

[73] Assignee: Toray Industries, Inc., Tokyo, Japan

[22] Filed: May 4, 1972

[21] Appl. No.: 250,176

[30] Foreign Application Priority Data

July 12, 1971 Japan..... 46-51092

[52] U.S. Cl..... 57/160, 28/1.4, 28/72.12, 57/34 B, 57/140 BY, 57/157 F

[51] Int. Cl. .... D02g 1/16, D02g 3/04, D02g 3/36

[58] Field of Search..... 57/157 F, 34 B, 140 BY, 57/140 R, 157 R, 160, 163, 58.95; 28/1.2, 1.3, 1.4, 72.12

[56] References Cited

UNITED STATES PATENTS

|           |         |                     |            |
|-----------|---------|---------------------|------------|
| 2,985,995 | 5/1961  | Bunting, Jr. et al. | 57/157 F X |
| 3,043,088 | 7/1962  | Breen               | 57/157 F   |
| 3,070,950 | 1/1963  | Thomas              | 57/163 X   |
| 3,137,991 | 6/1964  | Fairley             | 57/157 R X |
| 3,161,011 | 12/1964 | Humphreys           | 57/140 BY  |

|           |         |                  |            |
|-----------|---------|------------------|------------|
| 3,188,790 | 6/1965  | Hebeler          | 57/157 R X |
| 3,296,785 | 1/1967  | Hardy            | 57/157-R X |
| 3,474,613 | 10/1969 | Joarder et al.   | 57/157 F X |
| 3,603,043 | 9/1971  | Paliyenko et al. | 57/157 F X |
| 3,604,194 | 9/1971  | Edagawa et al.   | 57/58.95 X |
| 3,609,834 | 10/1971 | Lamb et al.      | 28/1.4     |
| 3,665,567 | 5/1972  | Clarkson         | 28/72.12 X |
| 3,672,147 | 6/1972  | Callieri et al.  | 57/157 F   |
| 3,678,549 | 7/1972  | Buzano           | 57/157 F X |

Primary Examiner—John W. Huckert

Assistant Examiner—Charles Gorenstein

[57] ABSTRACT

A yarn having soft, attractive handle and a structure such that staple fibers are intertwined with each other to cohere into a substantially non-twist yarn. The yarn is manufactured by supplying a substantially non-twist strand of staple fibers to a fluid treatment zone where the staple fibers are intertwined with each other by the turbulent flow, at least part of said staple fibers to be supplied to the treatment zone having a length larger than the distance L between the fiber grasping point in the fiber feed zone and the point where the intertwining due to the turbulent flow most effectively occurs.

10 Claims, 24 Drawing Figures



PATENTED JUL 9 1974

3,822,543

SHEET 01 OF 11

Fig. 1A



Fig. 2A



Fig. 3



Fig. 4



PATENTED JUL 9 1974

3,822,543

SHEET 02 OF 11

*Fig. 1B*



*Fig. 2B*



PATENTED JUL 9 1974

3,822,543

SHEET 03 OF 11

Fig. 5



Fig. 6



PATENTED JUL 9 1974

3,822,543

SHEET 04 OF 11

Fig. 7



Fig. 8



PATENTED JUL 9 1974

3,822,543

SHEET 05 OF 11

Fig. 9



Fig. 10



PATENTED JUL 9 1974

3,822,543

SHEET 06 OF 11

Fig. 11



Fig. 12



PATENTED JUL 9 1974

3,822,543

SHEET 07 OF 11

Fig. 13



Fig. 14



PATENTED JUL 9 1974

3,822,543

SHEET 08 OF 11

Fig. 15



Fig. 16



PATENTED JUL 9 1974

3,822,543

SHEET 09 OF 11

Fig. 17



Fig. 18



PATENTED JUL 9 1974

3,822,543

SHEET 10 OF 11.

Fig. 19



Fig. 20



PATENTED JUL 9 1974

3,822,543

SHEET 11 OF 11.

Fig. 21



Fig. 22



## SPUN-LIKE YARN AND METHOD OF MANUFACTURING SAME

The present invention relates to a novel non-twist high bulky yarn having a spun-like handle or feeling and a method of manufacturing the same. The novel bulked yarn has no substantial twist but a characteristic structure such that individual staple fibers are entangled with each other, which structure quite differs from conventional spun yarns and filament yarns, and is of high practical value.

Many methods for imparting high bulkiness to yarns are known wherein a raw yarn is fed into a fluid treatment zone where individual single strands are slackened and looped to form a bulky yarn thereby. For example, a typical method involves the steps of twisting a multifilament yarn and then making the twisted yarn pass through a fluid treatment zone under a slack state where the individual single filaments are looped by the turbulent flow to form a bulky yarn.

However, the twisting needs to be effected either before a multifilament yarn is subjected to fluid treatment as in the preceding method or after being subjected to fluid treatment, in order to set and make permanent the loops or the slacks formed through the fluid treatment. The need of twisting is obviously disadvantageous from an industrial viewpoint.

Also a method is known wherein a spun yarn is fed into a fluid treatment zone where the staple fibers are looped or slackened. However, a spun yarn usually has a relatively hard twist and therefore, the bulkiness is not remarkably improved even when subjected to the fluid treatment. Further, it is similarly disadvantageous that a spun yarn necessitates twisting for the preparation thereof.

It is the main object of the present invention to obviate the defects as mentioned above and to provide a substantially non-twist high bulk yarn having soft, appealing handle.

In accordance with the present invention, there is provided a yarn having a handle like spun yarn comprising staple fibers characterized by having a structure such that individual staple fibers are intertwined with each other to cohere thereby into a thread of high bulk having no twist on the whole. The novel yarn has a characteristic structure distinguished from conventional spun yarns, i.e. it is of very high bulk, assumes the peculiar form such that many end portions of the staple fibers project out of the periphery of the yarn as relatively long fluffs, and has no twist on the whole.

The yarn of the present invention will be illustrated in detail with reference to the drawings.

FIGS. 1A and 1B are a diagrammatical view and a photograph of a yarn of the present invention, respectively.

FIGS. 2A and 2B are a diagrammatical view and a photograph of another yarn of the present invention, respectively.

FIG. 3 is an explanatory view of the manufacture of the yarn shown in FIGS. 1A and 1B.

FIG. 4 is an explanatory view of the manufacture of the yarn shown in FIGS. 2A and 2B.

FIGS. 5 and 6 are a diagrammatical view of a fluid treatment apparatus used for the manufacture of the yarn of the present invention and an enlarged diagrammatical view of a bending part of the apparatus, respectively.

FIGS. 7, 8, 9 and 10 are diagrammatical views of other fluid treatment apparatus each used for the manufacture of the yarn of the present invention.

FIGS. 11 and 12 are diagrams showing relationships of the degree of intertwinement vs. difference in peripheral speed between feed rollers (front rollers) and delivery rollers, and of yarn strength vs.  $l/L$  ratio defined later, respectively.

FIGS. 13, 14, 15 and 16 are diagrammatical views of other fluid treatment apparatus each used for the manufacture of the yarn of the present invention further involving a second fluid treatment device.

FIGS. 17, 18, 19, 20 and 21 are diagrammatical views of other fluid treatment apparatus each used for the manufacture of yarns of the present invention involving the additional employment of a false twist system.

FIG. 22 is a diagram showing relationship of degree of intertwinement vs. the ratio of fiber diameter ( $d$ ) to mesh size ( $D$ ) of a deflecting member with perforations such as a screen used as a supplementary board for the intertwinement.

With reference to FIG. 1A diagrammatically showing the appearance of the yarn of the present invention, staple fibers 2 are intertwined with each other to cohere thereby into a single yarn 1 as though spun. The yarn 1 comprises loops 4 therein giving a very high bulk and fluffs 5 of relatively great length projecting out of the periphery thereof, which structure cannot be found in conventional spun yarns.

30 A method of manufacturing such a yarn will be described in detail:

The method involves the step of feeding a substantially non-twisted strand of staple fibers such as a roving or sliver from a fiber supply zone to a fluid treatment zone where individual staple fibers are intertwined with each other by a turbulent flow of fluid to cohere thereby into a single yarn, at least some of said staple fibers to be supplied to said fluid treatment zone have a length larger than the distance  $L$  between the grasping point in the fiber feed zone and the intertwining point in the fluid treatment zone. The term "intertwining point" means herein the point at which the intertwining of staple fibers most effectively occurs due to the turbulent flow in the fluid treatment zone.

50 In order to manufacture the yarn of the present invention, it is insufficient merely to subject a conventional non-twist strand of staple fibers to normal fluid treatment, i.e. it is necessary to employ specific conditions for intertwining the staple fibers with each other to a considerable degree. It is, therefore, fundamentally required that the fluid exerts a strong intertwining action on the staple fibers and that at least some of the staple fibers have a length larger than the above-specified distance.

55 FIG. 3 illustrates the principle of the method of the present invention. With reference to FIG. 3, a roving 7 unwound from a bobbin 6 is drawn, for example, approximately 20 times its original length while passing through back rollers 8, draft means 9, and front rollers 10, to become a non-twist strand in the form of fleece. The fleecy strand is continuously supplied from the front rollers 10 to a fluid treatment apparatus 12 through an inlet tube 11. High pressure fluid such as compressed air is introduced following the arrow through an inlet 13 into a disturbance chamber 14 and discharged through an outlet 15. An aspirator effect is

therefore produced on the inlet tube 11, whereby the fleecy strand is sucked into the disturbance chamber 14 and discharged therefrom through the outlet 15. In the fluid treatment zone, the individual staple fibers are actively intertwined with each other to form a single spun yarn 16 by the turbulent flow produced in the disturbance chamber 14 and the wide flow of fluid ejected through the outlet 15. The spun yarn 16 so formed is continuously wound into a package 18 by way of a take-up roller 17.

The feed stock, i.e. a strand of staple fibers such as a roving or sliver should comprise staple fibers lying substantially parallel at least some of which have a length  $L'$  larger than the distance  $L$  between the grasping point of the pair of front rollers 10 and the outlet 15 of the fluid treatment nozzle 14, i.e. the point at which the intertwining due to the turbulent flow most effectively occurs.

When all the staple fibers of the strand to be treated substantially have a length smaller than the distance  $L$ , the individual staple fiber escapes from the grasp of the front rollers before the forward end thereof reaches the outlet of the fluid treatment nozzle. Consequently, they are insufficiently intertwined with each other and some of them are scattered out from the outlet 15. It is difficult to produce a continuous yarn from such staple fibers.

In contrast, when at least a substantial number of the staple fibers have a length  $L'$  larger than the distance  $L$ , the staple fiber is still grasped between the pair of front rollers when the forward end thereof reaches the outlet and consequently, strongly intertwined with other staple fibers by the turbulent flow of the fluid to form thereby a continuous spun yarn.

It is noted however that the strand containing an excess of staple fibers having the length  $L'$  results in a spun yarn of reduced bulk and softness. Therefore, the ratio of the staple fiber having length  $L'$  contained in the strand should preferably be within a stated range, i.e. from 5 percent to 80 percent based on the total weight of the strand.

The fluid treatment apparatus where staple fibers are intertwined with each other to form a spun yarn of the present invention is not critical. Any type of fluid treating apparatus may be used as long as it is capable of exerting a sufficient intertwining action on the staple fibers. In particular, those of the type equipped with a jet apparatus capable of producing a strong turbulent flow such as, for example, of the type provided with two or more jet apparatus whereby two or more flows of fluid are simultaneously introduced into the fluid treatment zone as illustrated later, are preferred. Some conventional apparatus used for the production of filament yarn of high bulk by employing a fluid ejection technique may be used if the fluid treatment conditions are strictly determined.

The fluid used in the present invention may be either gas or liquid. Compressed air is most preferable because of ready availability and no baneful effect on the human body or the apparatus, and particular protection apparatus is not required. Hot air or saturated steam or super-heated steam may be preferably used when thermoplastic staple fibers are treated. Pressure of the fluid flow may be optionally varied.

Regarding the ratio in peripheral speed of the front rollers as a fiber supply source to the take-up roller, it may be varied depending upon the characteristic of sta-

ple fibers used, the material and form of staple fibers. The ratio is usually 1:1. It is however preferred to adjust suitably the ratio depending upon the particular spinning condition when a smooth treatment cannot be effected at the fixed ratio of 1:1 in the case where staple fibers having no crimp or having conventional crimp are used. The ratio may be varied in a manner such that some of the staple fibers are either strained or released during the treatment.

10 In a modified embodiment, a deflecting member (not shown in FIG. 3) is so arranged in front of the outlet 15 that the member deflects the fluid flow passing out of the outlet and consequently produces a further turbulent flow and enhances the intertwining effect of staple fibers. The distance between the deflecting member and the outlet may be suitably determined depending upon the desired spun yarn and the feed stock used.

15 The length of fluffs 5, i.e. end portions of the staple fibers projecting out from the periphery of the spun 20 yarn may be varied by altering the distance  $L$  between the grasping point of the front rollers and the outlet of the fluid treatment nozzle or the ratio in diameter of the inlet tube 11 to the thickness of the fleecy strand. That is, the length of fluffs increases with an increase 25 of the distance  $L$  and an increase of the ratio in diameter of the inlet tube to the thickness of the fleecy strand, and decreases with a decrease of these quantities. The length of fluffs may also be varied by varying the shape of crimp, surface characteristic and physical 30 characteristic of the staple fiber and the particular additives applied to the staple fiber.

The method of the present invention can be employed in the manufacture from both a non-twist strand of staple fibers and a filament yarn as well as the strand 35 of staple fibers alone. FIGS. 2A and 2B shows yarn manufactured from both staple fibers and filaments.

In this embodiment, as shown in FIG. 4, filaments 31 40 unwind from a bobbin 6' are supplied through guides 64 and a tension device 63 to a pair of front rollers 10 where the filaments are joined together with a fleecy strand 7 of staple fibers fed from a bobbin 6 through back rollers 8 and aprons 9 as illustrated referring to FIG. 3, and supplied into the fluid treatment nozzle 12. Alternatively, filaments 31 45 may be supplied into the fluid treatment nozzle 12 separately from the fleecy strand 7 of staple fibers.

The method of manufacturing the yarn of the present invention having handle like a spun yarn, will be illustrated in more detail with reference to the preferred 50 embodiments:

As briefly mentioned before, it is preferred to supply a substantially non-twisted strand of staple fibers to a fluid treatment zone provided with two or more fluid jets, i.e. to make the fleecy strand pass through two or 55 more fluid jets. The two or more fluid jets exert synergistically the intertwining action on staple fibers. The two or more fluid jets may be applied simultaneously or in sequence to staple fibers.

60 FIG. 5 shows one preferable embodiment of the fluid treating apparatus, wherein two paths for fluid are provided, one (shown in the right hand) being slopewise formed at a certain angle to the other (shown in the left hand) at the one end thereof and hence the two forming a crooked path.

65 In FIG. 5, a non-twist strand 7 is supplied from a fiber supply source comprising rollers with aprons 9 and front rollers 10 to a fluid treatment apparatus 14 where

the strand 7 is subjected to fluid treatment, and the resulting yarn 16 is delivered by way of a pair of delivery rollers 27. The fluid treatment apparatus 14 comprises a fiber inlet tube 11, a first fluid inlet tube 13, a fiber transportation tube 20, a second fluid inlet tube 26 and a slanting tube 22. Fluid, particularly compressed air, is introduced thereinto through the first and second fluid inlet tubes 13 and 26 at the same time. One end of the fiber transportation tube 20 is connected to the slanting tube 22, the longitudinal axis of which is in the direction of air flow through the second fluid inlet tube 26. The wall of the connecting portion of the fiber transportation tube 20 and the slanting tube 22, against which wall the air flow passing through the tube 20 runs, is provided with perforations of suitable number and size extending parallel to the axis of the fiber transportation tube 20. The strand 19 (i.e., the portion of the strand 7 in the fluid treatment zone) is subjected to the turbulent flow of air at the connecting portion where staple fibers are intertwined with each other to form thereby a single yarn. More particularly, the strand 19 passing together with the first air flow through the fiber transportation tube 20 intersects with the second air flow from the second fluid inlet 26, at the connecting portion, from which staple fibers, while being drawn to the wall provided with the perforations, are transported to the outlet of the tube 22 due to the second air flow and drawn out as a non-twist spun yarn by way of the delivery rollers 27. Preferably, a deflecting member 23 provided with perforations is arranged in front of the outlet of the slanting tube 22, i.e. at a point immediately downstream from the outlet whereby the air flow 25 and the output strand 16 of staple fibers at least a substantial number of which have been intertwined with each other are advantageously separated.

The intertwining effect produced at the point of intersection 24 of both the air flows as mentioned above will be illustrated in detail referring to FIG. 6, which diagrammatically shows an enlargement of the neighbourhood of the point of intersection.

The strand of staple fibers 19 passing through the fiber transportation tube 20 is intertwined therein to a certain extent. It is however not yet in the condition capable of forming a single yarn. The two air flows run against each other at the intersection point 24 and produce a turbulent flow whereby staple fibers are in complicated motion and are intertwined with each other to a greater extent. A part or a substantial part of the air flowing out of the fiber transportation tube 20 is discharged through perforations 21 made on the wall of the slanting tube 22 into the atmosphere. The yarn indicated by the numeral 28 in this region as spun is transported, accompanying the air flow introduced from the fluid inlet tube 26, through the slanting tube 22 to the outside.

In FIG. 5, the distance L mentioned before is defined as that between the grasping point of the front rollers 10 and the intersection point 24 of the two air flows, the latter point being the one at which the intertwinement of staple fibers most effectively occurs due to the turbulent flow.

FIG. 7 shows another preferred embodiment of the fluid treatment apparatus used in the present invention, involving two fiber supply sources; a non-twist fleecy strand of staple fibers and a filament yarn comprising a plurality of continuous filaments. Of course, filaments

may be additionally supplied to the fluid treatment apparatus of the type shown in FIGS. 5 and 6, for example, onto the strand of staple fibers at the upstream or downstream of the front rollers. It is however preferable to employ such an apparatus of the type as shown in FIG. 7 in order to treat both staple fibers and filaments.

Referring to FIG. 7, a non-twist strand of staple fibers 7 is supplied from a pair of front rollers 10 into a first fiber inlet tube 11 in the same manner as illustrated referring to FIG. 5 and simultaneously, a filament yarn 31 is supplied from a pair of front rollers 30 to a second fiber inlet tube 11' diverging from a fiber transportation tube 20. The fluid treatment apparatus 14 is similar to that shown in FIG. 5 except that the fiber transportation tube 20 is equipped with the filament yarn inlet and transportation tube 11' diverging therefrom at an angle of  $\theta^{\circ}$  and the latter tube 11' is connected to a slanting tube 22.

20 The intertwinement between the filament yarn 31 and staple fibers 7 is effected at the intersection point 34 of the fiber transportation tube 20 and the filament inlet tube 11' by a first fluid flow introduced from an inlet 13. Since the filaments 31 and the staple fibers 7 are intertwined while intersecting at an angle of  $\theta^{\circ}$ , the staple fibers sufficiently pierce the filament yarn. Further, a turbulent flow occurs as the first fluid accompanied with the intertwined fibers runs against the wall of the slanting tube 22, and therefore, enhances the intertwining effect on the fibers. Therefore, this embodiment is obviously preferred to that shown in FIG. 5 in the case where both a strand of staple fibers and a filament yarn are treated. In addition, a second fluid flow from a fluid inlet tube 26 enhances still more the intertwining effect. The distance L mentioned above is defined as that between the grasping point of the front rollers 10 and the intersection point 34 herein.

FIG. 8 shows a preferred embodiment similar to that of FIG. 7 except that two fluid flows are separately introduced into the apparatus 14 in the neighbourhoods of the two fiber supply sources, respectively. The two fluid flows from two fiber transportation tubes 20 and 20' impinge on each other at the intersection point 34 of the two tubes 20 and 20' and consequently, produce a very complicated fluid stream whereby individual staple fibers and filaments are strongly intertwined will each other to form a complete whole, a spun yarn with no twist.

50 The above-illustrated embodiments involve the use of two fluid flows separately directed to a strand of staple fibers. However, as a modified embodiment of the method involving the use of two or more fluid flows, the following type is enumerated wherein one fluid flow is directed to a strand of staple fibers twice in sequence, i.e. the strand once having passed out of the path of the fluid flow is turned back thereto:

That is, a strand of staple fibers is introduced into a fluid treatment apparatus having a fiber inlet tube and a fiber transportation tube and then, withdrawn from the apparatus to the vicinity thereof and again, turned back to the fiber transportation tube through which the strand passes countercurrentwise over a stated range, and finally withdrawn from a fiber outlet tube.

Referring to FIG. 9, a strand of staple fibers 7 is drawn through back rollers 8, a drafting element 9 and front rollers 10 into a fleece composed of staple fibers lying substantially parallel and then, introduced into a

fluid treatment zone in which a fluid treating apparatus 14, a deflecting member 23, a guide roller 35 and, a delivery roller 27 are arranged.

The fluid treatment apparatus 14 comprises a fiber inlet tube 11 and a fiber transportation tube 20 with which a slanting fiber transportation tube 22 is connected at a certain angle. The deflecting member 23 with perforations such as a screen is provided in front of one end of the slanting tube 22 in order to separate the intertwined fiber and the fluid. A fiber outlet tube 26 is provided at the other end of the slanting tube 22. In this arrangement, the distance L mentioned hereinbefore is defined as that between the grasping point of the front rollers 10 and the deflecting member 23. The distance between the deflecting member 23 and the intersecting point of the two fiber transportation tubes 20 and 22 is herein referred to as "l."

The strand 7 sucked into the fiber transportation tube 20 runs against the deflecting member 23 and then, is turned back to the tube 22 through which the strand passes countercurrently over a length of l, and withdrawn from the outlet 26 by way of the guide roller 35.

It has been found in the practice of the above-mentioned method that the difference ( $V_{01} - V_{02}$ ) between the speed of the fluid flow ( $V_{01}$ ) and the take-up speed ( $V_{02}$ ) of the yarn as spun, both in the course of yarn-formation over the range of l, and the ratio of  $l/L$  seriously affect the intertwining effect. Experimental results regarding these important factors are shown in FIGS. 11 and 12.

FIG. 11 shows the relationship between the difference in speed,  $V_{01} - V_{02}$  (expressed in m/min) and degree of intertwinement (expressed in number of cycles). On this experiment, both a strand of staple fibers and a filament yarn were simultaneously introduced into the apparatus shown in FIG. 9, and the degree of intertwinement between the stple fibers and between the staple fibers and the filaments was determined. The degree of intertwinement is determined in the following manner: One end of a yarn as spun is secured in one of the clamps and a pre-tensioning load of 10 mg/d is applied to the other end. The yarn is rubbed with a 1 mm diameter piano wire strung in the direction perpendicular to the single yarn by making the wire reciprocate. The number of cycles is noted when all the staple fibers fall out from the filaments. FIG. 12 shows the relationship between the ratio  $l/L$  and tensile strength of yarn (g/d). In this experiment, only a strand of staple fibers was treated with air using the apparatus shown in FIG. 9, and the tensile strength of yarn was determined as a measure of the degree of intertwinement.

As evident from FIGS. 11 and 12, a desired effect can be produced when the difference in speed,  $V_{01} - V_{02}$  is larger than  $0.75 \times 10^3$  m/min and the ratio  $l/L$  is larger than 0.25.

Referring to FIG. 10 illustrative of another modified embodiment of the method of the present invention, a strand 7 of staple fibers supplied from front rollers 10 passes through a fiber inlet tube 11 and a fiber transportation tube 20 and runs against a deflecting member 23 where only air flow passes through perforations thereof (following the arrows) and the yarn 37 as spun is turned back. The yarn 37 goes back through the tube 20 and is withdrawn from an outlet 26. The fluid treatment apparatus 14 is provided with a partition strip 38

having perforations whereby spinning stability can be ensured.

Further, it has now been found that the following method produces still more complicated turbulent flow and far enhances the intertwining effect; plural fluid flows are blown against a strand of staple fibers from the periphery thereof, while the staple fibers are suspended in the other fluid flow and intertwined with each other, in a manner such that the plural fluid flows are directed at a certain angle, e.g. perpendicular to and envelops the latter fluid flow.

Several preferred embodiments of the method are illustrated with reference to FIGS. 13 - 16.

Referring to FIG. 13, the fluid treatment apparatus 14 is provided with a second fluid treatment apparatus 42 at the intermediate portion of the fiber transportation tube 20, the latter apparatus 42 comprising a compressed air inlet 43 and plural spouts 44, 45, 46 and 47 disposed on the periphery of the fiber transportation tube 20. Compressed air is introduced through the inlet 43 into the apparatus 42 and blow through the plural spouts 44, 45, 46 and 47 against a strand of staple fibers from the periphery thereof while the staple fibers suspended in the first air flow are intertwined with each other, whereby the intertwining effect is suddenly increased due to the turbulent flow. The strand of staple fibers so intertwined passes out of the slanting portion 22 of the transportation tube, runs against a deflecting member 23 and then, is taken up by means of delivery rollers 27. In this embodiment, the intertwinement occurs most effectively at the point where the second plural air flows are blown against the strand and therefore, the distance L is defined as shown in FIG. 13. Instead of the second fluid flows being directed perpendicular to the first fluid flow supporting staple fibers, the second fluid flows or at least a part may be directed at some angle other than a right angle to the first fluid flow.

In the practice of the fluid treatment using the apparatus of the type as shown for example in FIG. 13, the first fluid flow interferes with the second fluid flow occasionally causing a backward flow of the first fluid. This phenomenon depends upon the volume rate of both fluid flows. It causes unevenness of yarn, reduction of the yarn strength and reduction of the suction force for the strand resulting in lowering of the treatment efficiency. Consequently, the volume rate of both fluid flows cannot be voluntarily increased.

In order to obviate such defects, it is preferred to provide one or more vents, in the wall of the fiber transportation tube between the first fluid feed zone and the second fluid feed zone whereby a part of the first fluid can escape from the system for the relief of pressure, as shown in FIG. 14.

In FIG. 14, orifices shown with numerical reference 48 are those mentioned above and other members are similar to those illustrated in FIG. 13.

Another example of the type as mentioned above is shown in FIG. 15. Referring to FIG. 15, the fiber transportation tube 20 is equipped at the slanting portion thereof with a second fluid treatment device 42 comprising spouts 46 and 47 and with orifices 48 as mentioned above at the crook thereof.

Referring to FIG. 16, the fiber transportation tube 20 is similarly equipped at the vertical portion thereof with a second fluid treatment device 42 comprising spouts 45, 46 and 47. But, instead of the orifices mentioned

above, an exhaust tube 49 having an inner diameter larger than that  $d$  of the fiber transportation tube is provided on the upper end of the vertical portion of the fiber transportation tube whereby a part of the first fluid can escape from the system.

Further, it has now been found that when a fiber cohesion treatment such as false twisting and alternate twisting is carried out together with the fluid treatment mentioned above, the intertwinement of staple fibers is far more enhanced and the surface configuration of the yarn becomes uniform. The fiber cohesion treatment may be carried out at any stage, e.g. before or after the fluid treatment or during the fluid treatment.

The fiber cohesion treatment taken just before the fluid treatment has the following advantages: (1) The grasping point of staple fibers in the fluid treatment as defined above is transferred from the front rollers to the point where the fiber cohesion treatment is carried out, e.g. false twisting point, that is the distance  $L$  is reduced and therefore, staple fibers of relatively short length can be used as a feed stock. (2) The cohesive attraction obviates undesirable scattering of staple fibers during the fluid treatment and enhances the intertwining effect far more. (3) Any kind of staple fiber can be smoothly supplied into the fluid treatment zone without varying the particular spinning conditions.

The fiber cohesion treatment taken after the fluid treatment has the following advantages: (1) The cohesive attraction improves uniformity of surface configuration of the yarn as spun and ties fluffs of a large length around the yarn proper, resulting in a yarn of high quality. (2) Since the cohesive attraction goes upstream to the fluid treating zone, first, staple fibers of relatively short length can be used which is similar to the former case where the fiber cohesion treatment is performed just before the fluid treatment, and secondly, the cohesive attraction unifies the motion of fibers and the intertwinement thereof and prevents the scattering of fibers, in the fluid treatment zone. Likewise, the fiber cohesion treatment taken during the fluid treatment produces the combined effects of those enumerated above. (3) Desirable characteristics in the yarn such as bulkiness and appearance (fluffs, loops and parallelism) is readily obtainable as the end use needs.

Members used for the fiber cohesion treatment include, for example, known spinners such as of the type used for false twist and alternate twist. Preferable spinners are a contact type spinner and a pneumatic vortex type spinner.

Several preferred embodiments of the apparatus involving the spinner are illustrated with reference to FIGS. 17 - 20. FIG. 17 diagrammatically shows an arrangement wherein a false twist spinner 50 is provided at the point immediately upstream of a fluid treatment apparatus 14. FIG. 18 shows an arrangement intended for practical use, wherein a fluid treatment apparatus 14 and a false twist spinner 50 are joined to each other through the medium of a bearing 52 and the false twist spinner 50 is driven by a suitable drive means 51. A false twist spinner can be similarly applied to all the fluid treatment apparatus shown in FIG. 5 and the following figures.

FIG. 19 shows an arrangement wherein a pneumatic vortex type false twist spinner 50 is provided at the point immediately downstream of the fluid treatment zone. In FIG. 19, a second fluid treating nozzle 42 is in-

tegrally equipped with the false twist member 50. A part of the compressed air from the inlet 43 of the second fluid treatment nozzle 42 is introduced through orifices 54 into a chamber of the false twist member 50 and blown out therefrom through orifices 53 eccentrically directed to the path of the yarn as spun whereby the yarn is false-twisted due to the air vortex. Alternatively, a false twist spinner of contact type may also be employed.

In FIG. 19, a fiber inlet tube 11 provided in a first fluid treatment nozzle 14 is slidable along the path of staple fibers and the distance between the fiber inlet tube 11 and a fiber transportation tube 20 may be varied by sliding the thumb head portion 58 thereof by hand, whereby the absorbing force in the first fluid treatment nozzle 14 can be suitably settled. The first fluid treatment nozzle 14 is connected with the second fluid treatment nozzle 42 by a connecting member 59.

In this embodiment, a strand of staple fibers passes through the fiber treatment zone under the following conditions:

As shown at the lower section of FIG. 19, the axis is drawn in parallel with the path of the strand of staple fibers, the origin being point O corresponding to the grasping point of the front rollers 10, and the points at which the strand is under action of the fluids, i.e. the fiber-feeding flow point the turbulent flow occurring point, the false twisting point and the point of collision with the deflecting member 23 are expressed as points P, Q, R and S, respectively. (The axis is also shown in FIG. 17.) If the apparatus is not equipped with the false twisting member 50, staple fibers undergo the action of the fluids in a nontwisted and nearly non-cohesive state at the section between the points O and Q' and intertwine with each other at the section between points Q' and R', as shown in the axis (a). On the contrary, in this embodiment of the present invention involving the employment of the false twisting member 50, staple fibers are under the false twist action at the section ranging from point O'' to point R'', as shown in the axis (b), and therefore, staple fibers undergo the action of turbulent flow in a false-twisted state at the section between Q'' and R''. That is, staple fibers are cohered together due to the false twist action immediately after passing the grasping point of the front rollers 10 and then, subjected to intertwinement in a considerably stable state at the section between Q'' and R'' to form a single yarn thereby. At the section downstream of point R'', the yarns so formed are in a substantially non-twisted state or a partially twisted state on rare occasions and run against the deflecting member 23 where the intertwinement is greatly enhanced, and then withdrawn therefrom as a substantially non-twist yarn.

FIG. 20 shows an arrangement wherein a contact type false twist spinner is provided at the point immediately downstream of the fluid treatment zone. The apparatus comprises a first fluid treatment nozzle 14 having a fiber inlet tube 11 and a fluid inlet tube 13, the nozzle having a sucking action on the strand of staple fibers, and a second fluid treatment nozzle 42 having a fiber transportation tube 20, a fluid inlet tube 43 and spouts 46, 47, the nozzle having an intertwining action on the strand of staple fibers, and a slanting tube 22 with perforations 21. Further, the apparatus comprises a false twist spinner 50 connected with the slanting tube 22. The false twist spinner 50 supported with a

support member 62 through the intermediation of bearings 52 is driven by a driving belt 51. The yarn as spun is therefore subjected to false twist by the contact with the inner wall of the spinner 50.

In this embodiment, a part of the fluid supporting the intertwined staple fibers is preferably withdrawn out through the perforations 21 whereby the yarn is smoothly subjected to false twist without disturbance.

As exemplified with reference to FIG. 20, when a yarn is subjected to false twist while passing through a contact-type tubular spinner, the peripheral surface of the yarn is kept in contact with the inner wall of the spinner over a stated length and therefore, excessively long fluffs are advantageously rolled up in the yarn proper, resulting in a yarn of uniform surface configuration.

FIG. 21 shows an arrangement wherein a pneumatic vortex type false twist spinner 50 is provided between the first fluid treating zone 14' and the second fluid treating zone 42'. The arrangement further involves vents 48 for the relief of pressure between the false twist spinner 50 and the second fluid treatment zone. This apparatus has a structure such that fluid supplied through one inlet 56 is distributed among the three treatment zones, i.e. through orifices 58 to the first fluid treatment zone 14, through orifices 57 to the false twisting zone and through orifices 45, 46, 47 to the second fluid treatment zone, which is obviously advantageous from the economical and efficient viewpoints.

In a modified embodiment of the apparatus with a spinner, a device serving both as a fluid treatment apparatus and a fiber cohesion treatment apparatus may be employed. For example, referring to FIG. 13, in the case where orifice 44, 45, 46 and 47 of the second fluid treatment apparatus 42 are eccentrically directed to the path of the strand, i.e. air flows therethrough are blown against the first air flow to form a vortex, false twist and the intertwinement can be simultaneously achieved.

In preferred embodiments of the present invention, a deflecting member having perforations such as a perforated board and a net as shown with numerical reference 23 in FIGS. 5, 7-10, 13-15 and 17-20 is employed which is placed at the point immediately downstream of the outlet of the fiber transportation tube. When a fluid flow carrying the strand of staple fibers runs against the deflecting member, a part of the fluid flow is deflected backwardly therefrom to form backward flows which open the strand and intertwine the staple fibers, and simultaneously a substantial part of the fluid flow passes through the perforations which makes the staple fibers slacken and loop. Further, isolated staple fibers, which would inevitably scatter therefrom without the deflecting member, temporarily stay thereon and are caught by the strand of staple fibers to form a part of the yarn. Consequently, the deflecting member provides an increase in the yield of the yarn as well as enhancement of the intertwinement between fibers.

The deflecting member should function such that the greater part of the fluid running against it passes through it. It has been found that the ratio (t) of the diameter (D) of the staple fibers to the diameter (d) of perforations in the deflecting member has a close relation to the degree of the intertwinement and, for satisfactory results, should be within the range:

$$4 < t = (d/D) < 500.$$

The shapes of both the perforations and the cross-section of the fibers are not critical; circular or any other shapes may be employed as long as the diameter of the inscribed or circumscribed circle satisfies the above inequality.

FIG. 22 shows the relation between the ratio in diameter ( $t = d/D$ ) and the degree of intertwinement (number of cycles, determined by the procedure hereinbefore described), resulting from the experiments wherein a roving of nylon staple fibers having a fineness of approximately 1.5 denier ( $D \approx 12 \mu$ ) and various deflecting members with perforations differing from each other are employed.

The yarn obtained in accordance with the method of the present invention may be additionally finished, for example, by making the yarn contact a rotating member whereby fuzz is prevented or rolled up into the yarn proper without or with applying heat thereto in order to set the yarn, if desired.

In accordance with the present invention, various kinds of substantially non-twist yarns having handle like a spun yarn can be obtained employing various staple fibers as a feed stock.

The staple fibers used as a feed stock are not critical; all kinds of staple fibers may be used such as synthetic fibers, cotton, wool, regenerated fibers and the like. Further, a single kind of staple fiber, a blend of staple fibers different from each other in the material, fineness, fiber length, cross-sectional configuration, crimp characteristics, elongation or the like may also be used. A blend of staple fibers different in characteristic or heat shrinkage may also be used. In the case where a blend of staple fibers different in fluid intertwining characteristics is used, the resulting yarn has an attractive cross section wherein both staple fibers are distributed in varying proportions ranging from the central portion to the peripheral portion. Further, in the case where a blend of staple fibers different in heat shrinkage is treated in accordance with the present invention, followed by heat treatment, the resulting fiber also has an attractive cross section wherein the proportions of both staple fibers in the central portion and the peripheral portion are different from each other.

Plural strands each comprising staple fibers different from those of the other may be separately supplied into the feed treatment zone. In this case, when the feed rate of each strand is intermittently varied, yarns of attractive appearance are obtainable, e.g., in a structure where different staple fibers are alternately arranged in the longitudinal direction or a structure where the yarn diameter is periodically varied.

In addition to one or more non-twist strands of staple fibers, one or more continuous filament yarns may be simultaneously or separately supplied into the fluid treatment zone as illustrated with reference to FIGS. 7-10. The filament yarn which becomes a core in the core spun yarn of the present invention, comprises for example a conventional synthetic filament yarn, its crimped yarn, a textured yarn, an elastomeric yarn, a flat yarn, a gold or silver thread, a glass yarn and a metallic yarn. Both multifilament and monofilament yarns may be used. When plural filament yarns are employed, the yarns are preferably treated with fluid in a completely opened state. In particular, when an elastomeric yarn made of elastomeric material such as polyure-

thane or a stretch yarn is employed, it is preferable to subject it to tensioned treatment or treatment under slack conditions prior to the fluid treatment to become opened thereby. Textured yarns as herein used mean those consisting of either non-elastic, continuous filaments or non-elastic staple fibers, both of which have been made stretchable through reformation for example by the heat-set coil, crimp or curl methods. It is further practicable that a latently crimped filament yarn or a strand of latently crimped staple fibers is subjected to the fluid treatment and then, heat-treated to develop crimps. When a core yarn is used, it is also practicable to subject the resulting yarn to tensioned treatment after the fluid treatment to straighten the core yarn component and hence, to make the yarn hold a firm appearance. Further, it is also practicable to twist the filament yarn before supplying it to the fluid treatment zone, to a certain extent e.g. less than 500 T/M whereby the intertwinement thereof with staple fibers is enhanced.

The yarn of the present invention is of high bulk and has a soft, attractive handle similar to that of conventional spun yarns. The characteristic structure such that individual staple fibers are intertwined with each other to cohere into a substantially non-twist yarn, is distinguishable from conventional yarns made due to cohesive attraction such as twist, or adhesion, melting or sticking together. In addition, the yarn of the present invention has the advantage of reduced surface lubrication since it has numerous fluffs of a relatively large length.

In the practice of the method for manufacturing the yarn of the present invention, there is no necessity to provide a high speed revolution member for twisting and therefore, the spinning speed may be increased to 200 m/min or more, for example.

The invention will now be described with reference to Examples.

#### EXAMPLE 1

A roving of polyacrylonitrile staple fibers (fineness of 3 d, length of 120 mm), having a yarn number of 0.7 g/m, was drawn 20 times its original length by a drafting means and then, fed through front rollers to the fluid treatment apparatus shown in FIG. 5.

The distance L between the grasping point of the front rollers (10) and the point where the intertwinement most effectively occurs was 80 mm. Pressure and flow rate of both first and second air flows were 3 kg/cm<sup>2</sup> and 150 l/min, respectively. Peripheral speed of both the front rollers (10) and the delivery rollers (27) was 200 m/min.

The yarn having a yarn number of one thirty-fourth Nm, so produced, exhibited an appearance as shown in FIGS. 1A and 1B and was of high bulk.

#### EXAMPLE 2

A roving was prepared by blending two polyacrylonitrile staple fibers of a fineness of 3 d and a length of 120 mm, one being of ordinary shrinkage and the other being of high shrinkage, in a proportion of 6:4, respectively. The roving of a yarn number of 1 g/m, so prepared, was drawn by a drafting means and then, supplied to a fluid treatment apparatus shown in FIG. 5. The distance L defined herein before was 80 mm. Compressed air having a pressure of 3 kg/cm<sup>2</sup> was introduced through two inlets 13 and 26 into the apparatus

14, each at a flow rate of 160 l/min. Peripheral speed of both front rollers 10 and delivery rollers 27 was 200 m/min.

The spun yarn having a yarn number of one thirty-fourth Nm, so produced, had numerous fluffs of lengths ranging approximately from 10 – 30 mm and exhibited superior fiber intertwinement and fiber cohesion.

The spun yarn was wound into hanks, and then subjected to steaming at a temperature of 110°C for 10 minutes under relaxed conditions to be made bulky thereby, and then rewound by a hank reeling machine. When it was rewound at the rate of 2 kg per reel, the yarn was smoothly unravelled and no yarn breakages could be observed.

#### EXAMPLE 3

A blended roving used in Example 2 and a polyamide multifilament yarn having a total fineness of 50 d and comprising 24 filaments were simultaneously supplied into the fluid treatment apparatus shown in FIG. 5. A core spun yarn of high bulk and softness was obtained.

#### EXAMPLE 4

A roving of polyacrylonitrile staple fibers having a fineness of 3 d and various lengths (average length of 150 mm and maximum length of 200 mm) was supplied to the fluid treatment apparatus shown in FIG. 5. The treatment conditions were as follows:

|                                                               |                        |
|---------------------------------------------------------------|------------------------|
| Peripheral speed (V <sub>1</sub> ) of the front rollers 10    | 149 m/min              |
| Peripheral speed (V <sub>2</sub> ) of the delivery rollers 27 | 127 m/min              |
| Take-up speed                                                 | 145 m/min              |
| Pressure of the air introduced through the inlet 13           | 3.0 kg/cm <sup>2</sup> |
| Pressure of the air introduced through the inlet 26           | 3.2 kg/cm <sup>2</sup> |
| Deflecting member                                             | a wire gauge           |
| Distance (L)                                                  | 70 mm                  |

The spun yarn having a yarn number of one-fourteenth Nm, so produced, was of very high bulk and had numerous fluffs, loosenings and loops.

In particular, when both peripheral speeds (V<sub>1</sub> and V<sub>2</sub>) of the front rollers and the delivery rollers satisfied the following inequality, most preferable results were obtained.

$$0.03 < (V_1 - V_2/V_2) < 0.5$$

#### EXAMPLE 5

Using a fluid treatment apparatus shown in FIG. 8, a roving of polyester staple fibers having a fineness of 2.5 d and various lengths (average length of 128 mm) and two polyester filament yarns each having a total fineness of 50 d and comprising 48 filaments were treated under the following conditions:

|                                                               |                        |
|---------------------------------------------------------------|------------------------|
| Peripheral speed (V <sub>1</sub> ) of the feed rollers        | 104 m/min              |
| Peripheral speed (V <sub>1'</sub> ) of the feed rollers 10'   | 106 m/min              |
| Peripheral speed (V <sub>2</sub> ) of the delivery rollers 27 | 87 m/min               |
| Pressure of the air introduced through the inlet 13           | 2.5 kg/cm <sup>2</sup> |

—Continued

Pressure of the air introduced through the inlet 13' 3.5 kg/cm<sup>2</sup>

Intersecting angle ( $\theta$ ) between the two air inlet tubes 13 and 13' 45° 5

Distance L 55 mm

Deflecting member a wire gauge

The yarn having a yarn number of 1/15.5 Nm, so produced, was a fancy one of very high bulk involving a suitable number of fluffs and loops. 10

Likewise, various yarns of unusual and attractive appearances were obtainable under varying conditions of feed speeds of both the roving and the filament yarn, 15 delivery speed and air pressure.

#### EXAMPLE 6

Using a fluid treatment apparatus shown in FIG. 9, a roving of polyacrylonitrile staple fibers having a fineness of 3 d and various lengths (average length of 128 mm) and two polyamide multifilament yarns each having a total fineness of 50 d and comprising 34 filaments were treated under the following conditions: 20

Over-feed rate in the air treatment zone 12%  
 Distance l 40 mm  
 Distance L 98 mm 30  
 Air pressure 4.0 kg/cm<sup>2</sup>  
 Speed of air flow ( $V_{01}$ ) at the vicinity of the outlet in the tube 22 1200 m/min  
 Peripheral speed of the delivery rollers 27 100 m/min 35

The peripheral speed of the delivery rollers 27 corresponds to the take-up speed ( $V_{02}$ ) defined hereinbefore, and hence ( $V_{01} - V_{02}$ ) was approximately  $1.1 \times 10^3$  (m/min). The ratio l/L was 0.4. 40

As illustrated above, the strand of staple fibers and the filament yarns are preferably overfed into the treatment zone. Most preferably, both peripheral speeds ( $V_1$  and  $V_2$ ) of the front rollers 10 and the delivery rollers 27 satisfy the following inequality: 45

$$0.03 \leq (V_1 - V_2)/V_1 \leq 0.50$$

The yarn, so produced, exhibited the following properties: 50

Yarn number 1/16.5 Nm  
 Tensile strength 1.5 g/d  
 Elongation 14% 55  
 Degree of intertwinement 35 cycles

The yarn was of very high bulk. In the case where the yarns were doubled and then false-twisted, the resulting yarn exhibited extremely reduced yarn unevenness and could be used for various articles of clothing. 60

#### EXAMPLE 7

Using a fluid treatment apparatus shown in FIG. 13, a roving of polyacrylonitrile staple fibers having a fineness of 3 d and various lengths (average length of 128 mm) was treated under the following conditions: 65

—Continued

Peripheral speed ( $V_1$ ) of the front rollers 10 120 m/min  
 Peripheral speed ( $V_2$ ) of the delivery rollers 27 107 m/min  
 Pressure of the air introduced through the inlet 13 4.0 kg/cm<sup>2</sup>  
 Pressure of the air introduced through the inlet 43 4.5 kg/cm<sup>2</sup>  
 Distance L 65 mm  
 Deflecting member 23 a wire gauge of 300 meshes

The spun yarn having a yarn number of 1/12.0 Nm, so produced, was of high bulk. The yarn exhibited strong intertwinement between the staple fibers although the yarn was not substantially twisted, and a considerably reduced unevenness, and was quite suitable for knitting. 25

It has been confirmed from further experiments wherein the ratio of  $V_1$  to  $V_2$  was varied that a satisfactory yarn is not obtainable unless  $V_1$  is larger than  $V_2$ .

#### EXAMPLE 8

Using a fluid treatment apparatus shown in FIG. 18, a blended strand of two kinds of polyacrylonitrile staple fibers of equal weight, one having a fineness of 3 d and various lengths (average length of 128 mm) and the other having a fineness of 5 d and various lengths (average length of 102 mm) was treated under the following conditions:

Peripheral speed ( $V_1$ ) of front rollers 10 150 m/min.  
 Peripheral speed ( $V_2$ ) of delivery rollers 132 m/min  
 Take-up speed 145 m/min  
 Number of revolutions of false-twist spinner 50 18,000 rpm  
 Pressure of the compressed air 4.0 kg/cm<sup>2</sup>  
 Deflecting member a wire gauge of 300 meshes

The yarn having a yarn number of 1/13.5 Nm, so produced, was of very high bulk and quite suitable for various knitted and woven goods. Its workability was excellent i.e. yarn breakage was only 15.5 times/1,000 sp. × hr. and yield was 97 percent. 50

#### EXAMPLE 9

Using a fluid treatment apparatus shown in FIG. 21, a roving of polyester staple fibers having a fineness of 1.5 d and various lengths (average length of 125 mm) was treated under the following conditions:

Peripheral speed ( $V_1$ ) of front rollers (not shown) 103 m/min  
 Peripheral speed ( $V_2$ ) of delivery rollers (not shown) 95 m/min  
 Peripheral speed of take-up roller (not shown) 104 m/min  
 Pressure of the air introduced through inlet 56 4.5 kg/cm<sup>2</sup>

$d$  and  $\theta_0$ ,  $\theta_1$  and  $\theta_2$ , 0.3 m/m, 30°, 20° and 15°, respectively.

The spun yarn having a yarn number of one-thirtieth Nm, so produced, was a fance one of high bulk with long fluffs. The apparatus used was superior in workability and it resulted in satisfactory yarns without a deflecting member.

#### EXAMPLE 10

A fluid treatment apparatus shown in FIG. 18 was used, but the false-twist spinner 50 was used without revolution. A roving of polyacrylonitrile staple fibers having a fineness of 3 d and various lengths (average length of 102 mm) was drawn by a drafting device into a fleecy strand and then, the strand was supplied to front rollers 10 of the apparatus. Simultaneously, a polyamide filament yarn having a total fineness of 70 d and comprising 13 filaments was unwound from a pirl and directly supplied to the front rollers 10. Spinning conditions were as follows:

|                                                                                             |                      |
|---------------------------------------------------------------------------------------------|----------------------|
| Peripheral speed ( $V_1$ ) of front rollers 10                                              | 105 m/min            |
| Peripheral speed ( $V_2$ ) of delivery rollers (not shown)                                  | 89 m/min             |
| $(V_1 - V_2)/V_1 = 0.15$                                                                    |                      |
| Distance L between front rollers 10 and deflecting member 23                                | 90 cm                |
| Pressure of the air introduced through inlet 13                                             | 4 kg/cm <sup>2</sup> |
| Diameter ( $d$ ) of perforations of deflecting member 23                                    | 300 $\mu$            |
| Content of staple fibers having a length larger than L in all the staple fibers (by number) | 5%                   |
| Ratio ( $t$ ) of $d$ to the diameter (D) of staple fiber                                    | 15                   |

The non-twist yarn having a yarn number of one-fourteenth Nm, so produced, was of very high bulk and had numerous fluffs like a plied spun yarn and a suitable number of loops and loosenings. The yarn had a degree of intertwinement of 24 cycles and was suitable for various knitted and woven goods.

#### EXAMPLE 11

Using a fluid treatment apparatus shown in FIG. 18 without driving the false-twist spinner 50, a roving of polyacrylonitrile staple fibers having a fineness of 5 d and various lengths (average length of 102 mm) and a polyurethane elastomeric filament yarn having a fineness of 40 d and an elongation of 370 percent were simultaneously treated under the following conditions, and then false-twisted.

|                                                                   |                        |
|-------------------------------------------------------------------|------------------------|
| Peripheral speed ( $V_1$ ) of front rollers 10                    | 140 m/min              |
| Peripheral speed ( $V_2$ ) of first delivery rollers (not shown)  | 125 m/min              |
| Peripheral speed ( $V_3$ ) of second delivery rollers (not shown) | 120 m/min              |
| Peripheral speed ( $V_4$ ) of take-up roller                      | 138 m/min              |
| Pressure of the air introduced through inlet 13                   | 4.2 kg/cm <sup>2</sup> |
| Distance L (defined in Example 10)                                | 130 mm                 |
| Number of false twists                                            | 1,100 T/m              |

The yarn having a yarn number of one-fourteenth Nm, so produced, had the structure such that the elastic filaments were covered with the strand of staple fibers wherein the staple fibers were intertwined with

each other and with the elastic filaments, and exhibited handle and appearance like plied spun yarn. Since most long fluffs were twined round the yarn proper, the yarn was superior in bulkiness and intertwinement and suitable for various articles of clothing.

In order to evaluate the yarn of the present invention, several characteristics of the yarn were listed in the following table in comparison with those of conventional spun yarns.

10

| Specimen                       | A     | B     | C     |
|--------------------------------|-------|-------|-------|
| Bulkiness (cm <sup>3</sup> /g) | 46.3  | 11.1  | 33.6  |
| Water absorption (%)           | 197.3 | 148.0 | 156.3 |
| Kink coefficient               | 0     | 45.7  | 28.4  |
| Flexural rigidity              | 0.37  | 0.31  | 0.35  |

20

Note: (1) Specimen

A. Spun yarn prepared in the manner described in Example 7.

B. Commercially available spun yarn having a number of twist of 200 T/m prepared by a ring spinning frame.

C. Textured yarn prepared from the above commercially available spun yarn by a Taslan bulking process using a conventional air treatment apparatus.

25

These specimen yarns had a yarn number of one-eleventh Nm and were prepared from polyacrylonitrile staple fibers.

#### (2) Determining procedure

##### (2) - 1 Bulkiness

30

Bulkiness is expressed as specific volume (cm<sup>3</sup>/g). A 100 turns of the specimen yarn is wound on a hank reel having a perimeter of 1 m. Four hanks so prepared are put together and then folded double, followed by tying a cloth tape round them. Specific volume of the specimen is determined by attaching a sinker thereto.

##### (2) - 2 Water absorption

35

Water absorption is a measure of the moisture holding capacity of the yarn, and defined by the following equation:

$$\text{Water absorption, per cent} = (W - W_0/W_0) \times 100$$

where:  $W_0$  = weight of the hank of specimen yarn conditioned in the standard atmosphere of 20°C and 65% RH.

40

$W$  = weight of the hank after immersion. After the hank is immersed in water at 20°C for 20 minutes, the hank is clamped at one end thereof. The yarn is weighed at the moment when water ceases to drip.

##### (2) - 3 Kink coefficient

45

A specimen yarn of 50 cm test length was clamped at both ends in a substantially horizontal disposition. Next, the distance between the clamps was narrowed until a kink developed on the yarn. The length ( $l$  cm) of the distance between the clamps at this kink development was measured, from which kink coefficient is calculated as follows:

$$\text{Kink coefficient} = l \times (100/50)$$

##### (2) - 4 Flexural rigidity

50

A hysteresis curve is drawn in rectangular coordinates the abscissa being the curvature ( $1/\rho$ ) and the ordinate being the bending moment of a specimen yarn. The inclines ( $\alpha$ ) at the intersecting points of the curve with the ordinate are calculated. Flexural rigidity is expressed as the including ( $\alpha$ ).

55

As is apparent from the above table, the yarn of the present invention has the following features:

1. The yarn is of very high bulk which is evident from the water absorption as well as the bulkiness. In gen-

eral, the yarn of the present invention exhibits a water absorption larger than 170 percent.

2. As is apparent from the kink coefficient, the yarn has no torque due to the twist. Therefore, there is no necessity to steam the yarn of the present invention, although conventional spun yarns particularly composed of synthetic fibers exhibiting a high torque necessitate such treatment.

3. As is apparent from the flexural rigidity, the yarn of the present invention exhibits superior resistance to bending although it has no substantial twist. Therefore, knitted and woven goods made therefrom are stiff and not limp.

What we claim is:

1. A method of manufacturing a yarn having handle like spun yarn characterized in grasping a substantially non-twist strand of staple fibers at a fiber grasping point, supplying said fibers from said point to a fluid treatment zone, intertwining said staple fibers with each other in said zone with a turbulent flow to cohere into a single yarn, at least some of said staple fibers supplied to said fluid treatment zone having a length larger than the distance between said fiber grasping point in the fiber feed zone and the point where the intertwinement due to said turbulent flow most effectively occurs in said fluid treatment zone whereby a substantially non-twist yarn is produced, part of said staple fibers forming loops and fluffs projecting out of the periphery of said yarn, and then running the non-twist yarn accompanying a fluid flow against a deflecting member with perforations through which a substantial part of the fluid flow passes, whereby the intertwinement between the staple fibers and the formation of the loops and the fluffs are enhanced.

2. A method as claimed in claim 1 further characterized in that at least two fluid flows are blown against said substantially non-twist strand of said staple fibers in said fluid treatment zone whereby said staple fibers are intertwined with each other.

3. A method as claimed in claim 2 further characterized in that a first fluid flow is blown against said strand

of said staple fibers and then, a second fluid flow is blown against said strand of said staple fibers while said staple fibers are suspended in and transported by the first fluid flow in a partially intertwined state.

5 4. A method as claimed in claim 3 further characterized in that said second fluid flow is blown against said strand of said staple fibers from a direction inclined to the course of said first fluid flow suspending and transporting said strand of said staple fibers at which intersection point said staple fibers alter their course and are suspended in and transported by the second fluid flow.

10 5. A method as claimed in claim 3 further characterized in that said second fluid flow to be blown against said strand of said staple fibers suspended in and transported by said first fluid flow in a partially intertwined state is a vortex flow.

15 6. A method as claimed in claim 3 further characterized by venting said first fluid flow accompanied by said strand of the staple fibers for the relief of pressure, between two points at which said first fluid flow and said second fluid flow are blown against said strand of the staple fibers, respectively.

20 7. A method as claimed in claim 1 further characterized in that said strand of said staple fibers, after said staple fibers are at least partially intertwined with each other in the fluid treatment zone and withdrawn therefrom while being suspended in the fluid flow, is turned back and made to pass countercurrentwise through said fluid flow.

25 8. A method as claimed in claim 1 further characterized in that said strand of said staple fibers is subjected to alternate twisting before the fluid treatment.

30 9. A method as claimed in claim 1 further characterized in that said substantially non-twist strand of said staple fibers is supplied together with a continuous filament yarn to the fluid treatment zone.

35 10. A method as claimed in claim 1 further characterized in that said strand of said staple fibers is subjected to alternate twisting during the fluid treatment.

\* \* \* \* \*

UNITED STATES PATENT OFFICE  
CERTIFICATE OF CORRECTION

Patent No. 3,822,543 Dated July 9, 1974

Inventor(s) Hiroshi Edagawa, et al

It is certified that error appears in the above-identified patent and that said Letters Patent are hereby corrected as shown below:

Column 6, Line 46: "will" should be --with--

Column 8, Line 21: "blow" should be --blown--

Column 14, Line 52: " $0.03 < (V_1 - V_2/V_2) < 0.5$ " should be

$$\frac{0.03 < V_1 - V_2 < 0.5}{V_2}$$

Column 17, Line 2: "fance" should be --fancy--

Column 18, Line 41: " $(W - W_0/W_0) \times 100$ " should be

$$\frac{W - W_0}{W_0} \times 100$$

Signed and sealed this 17th day of December 1974.

(SEAL)  
Attest:

McCOY M. GIBSON JR.  
Attesting Officer

C. MARSHALL DANN  
Commissioner of Patents